

## UNITED STATES PATENT OFFICE

2,229,357

## FIBROUS PRODUCT

Gordon E. Wightman, Upper Montclair, N. J., and Ernest Kitzmacher, Manchester, Conn., assignors, by mesne assignments, to Union Carbide and Carbon Corporation, New York, N. Y., a corporation of New York

No Drawing. Application January 25, 1937,  
Serial No. 122,312

3 Claims. (Cl. 92—40)

This invention relates to the production of paper or other fibrous sheet material having a resinous substance associated therewith for the purpose of increasing the resistance of the material to moisture, and is particularly directed to a new method of producing such material and to the novel products thereby produced.

One of the purposes of the invention is to provide a method of effectively associating a resinous substance with the fibers of paper or like material.

It is known to treat paper and like material with rosin to impart water resistance thereto. The usual practice is to add to the wet fibrous pulp a rosin soap made by boiling rosin with sodium carbonate. After mixing the rosin soap with the pulp the rosin is precipitated by the addition of alum and the pulp is then formed into a sheet or board and dried.

It has also been proposed to dissolve rosin in a solvent immiscible with water, such as carbon tetrachloride, and apply the solution to the pre-formed sheet, after which the solvent is removed therefrom.

The first method entails the disadvantage that the addition of alum to effect precipitation of the rosin results in the presence of free acid which injures the fibers. The second method requires the drying of the sheet before it can be treated with the rosin solution, and a subsequent drying operation is required for removing the solvents from the sheet. Apparatus for recovering the solvent is also required. A further disadvantage of this method is that the solvents tend to carry the solute to the surface of the sheet and concentrate it there upon evaporation.

These disadvantages are eliminated by the present invention which comprises the treatment of the web of paper or other fibrous material with resinous substances or compositions in the form of clear aqueous dispersions which are dilutable with further quantities of water. These resinous compositions are apparently not true aqueous solutions since there is a limit to the amount of water which may be added without causing resin precipitation with attendant clouding of the dispersion. In general, the most satisfactory dispersions for use on wet paper pulp have been found to be those which will tolerate the addition of substantially more than an equal amount of water without initiating clouding or precipitation of the resinoid. In other words, a resin dispersion containing about 60% of resinoid will tolerate an additional quantity of water sufficient to give a clear unclouded resin disper-

sion of about 30% resin content. Generally speaking, resinous compositions of the character above described are spoken of as being hydrophilic or "water loving" in nature, but for the purposes of this invention, only those resinous compositions which will tolerate the addition of substantially more than an equal amount of water without becoming turbid or cloudy will be designated as hydrophile. It will be seen therefore that the hydrophile compositions utilized in the present invention are characterized by containing a resinous product capable of holding up to seventy parts of water per thirty parts of the resinous product, even in neutral condition.

A further distinguishing feature of these filterable hydrophile resinous compositions is the relatively small amount of resinoid migration which occurs in fibrous sheets treated with these compositions. Thus, when the volatile portion of the hydrophile resinous composition is removed, as for example by evaporation, the resinoid appears to remain in the form of adhesive films upon individual parts of or within the fibers themselves, instead of migrating to the exposed surfaces of the fibers, as is so often the case when organic solvent dispersions of comparable resinoid concentration are used.

Of particular value in the present invention are heat hardenable resinous substances or resinoids, especially those substances which change to a hydrophobe condition upon the application of heat so that, in the final heat treated condition, they are substantially unaffected by moisture. Especially suitable substances for use in the present invention are the liquid masses obtainable by reacting about equimolecular proportions of phenol or cresol with aqueous formaldehyde in the presence of a small amount, say 1 to 2% based on the phenolic constituent, of an alkaline or other suitable catalyst, stopping the reaction before there is any precipitation or separation of resinoid. The resulting relatively clear liquid dispersion will normally contain about 60% resinoid, and will tolerate the addition of substantially more than an equal amount of water without becoming cloudy or precipitating the resinoid. If a drop of the liquid is applied to a wet fibrous surface, it does not remain concentrated on the area to which it is applied, but immediately disappears into the mass of the sheet. Neither does it require a neutralizing or acidifying agent to deposit the resinoid.

A reaction product of the phenolic type can be made dilutable with water under operating conditions differing from the above, such as using a

smaller amount of alkaline catalyst and reacting for a longer period of time, or until the reaction mixture separates into two layers, and then adding up to 5-10% more of caustic based on phenol to obtain an aqueous solution, or a large amount of alkaline catalyst, say about 5-10% sodium hydroxide based on phenol, may be used in the initial reaction when a liquid mass results which can be diluted with water as desired. However, as the amount of caustic used is increased beyond 1 or 2% the mass appears to take on more and more the characteristics of a resinoid soap in solution, and at 4% or more, to exhibit the properties of true salt solutions to the extent of requiring precipitation or neutralization by known means such as alum to remove caustic present in excess of 4%, and preferably caustic in excess of 2% either before or after applying the resinous composition to the fibrous sheet.

20 In accordance with the present invention, therefore, it has been found that to avoid removal of caustic present in excess of 2% without resorting to precipitation or neutralization it is necessary to use not in excess of 2% of an alkaline catalyst during resin condensation, and moreover, that the condensation should be interrupted before there is any precipitation or separation of the resinoid.

It has been found, furthermore, that the aqueous mass need not be of an alkaline character. Instead the alkaline catalyst may be completely neutralized by sufficient acid and the neutralized solution may be used. Or a small amount of an organic acid such as phenol, tannic acid, citric acid, lactic acid, etc., can be added to give an acid reaction, and stable aqueous masses are thereby obtained which can be diluted with substantially more than an equal amount of water without clouding or precipitating the resinoid.

40 Typical examples for the preparation of hydrophile resinoids suitable for the purposes of this application are the following:

#### Example 1

45 100 parts of phenol and 80 parts of aqueous formaldehyde (40% solution) are reacted in the presence of 0.8 part sodium hydroxide for about 30 minutes. At the end of the reaction period, the liquid mass is still clear and no precipitation has occurred. It is dehydrated preferably in vacuo until the resinoid content formed constitutes about 60% of the total mass. The viscosity of the finished dispersion will be about 80-100 55 cp. If the liquid mass is diluted with an equal weight of water or until the resinoid content is about 30% it still remains clear and suitable for use with alpha cellulose fibers, pulp or ground wood.

60 When cresols or other higher phenols are used as a component of the resinoid, or when a more extended dilution with water is desirable, it is generally advantageous to include a volatile water-soluble organic solvent, such as alcohol, in the liquid mass to avoid precipitation of the resinoid. For example, if alcohol is present in an amount of about 10% of the water the composition may be diluted to a resinoid content of as little as 5% of the total mass. However, even 65 without the inclusion of an organic solvent the mass is not rendered unusable even by dilution until clouding occurs for the hydrophile property of distributing in water or spreading and disappearing when applied to a wet fibrous surface is still manifested.

#### Example 2

100 parts of cresol and 87.5 parts of aqueous formaldehyde (40% solution) and 5.3 parts ammonium hydroxide (28% solution of ammonia in water) are reacted 30 minutes at 90° C. The reaction mass is then dehydrated preferably in vacuum until a test portion of the resin is hard and brittle when dropped into water at 2° C. 5 73.7 parts of denatured alcohol are added to give a spirit varnish containing about 60% resinoid. Such a dispersion will have a viscosity of about 10 80-100 cp. 50 parts of this dispersion blended with 50 parts of the hydrophile resin described in Example 1 may be diluted with 100 parts of water to give a water-alcohol-resin dispersion 15 which is slightly opalescent but suitable for treating a web of paper or other fibrous material.

#### Example 3

145 parts of phenol, 145 parts formalin and 1 part sodium carbonate are reacted 1 hour under reflux. 0.75 part of concentrated sulfuric acid are added to the clear liquid and then 1 part of tannic acid, rendering the liquid mass slightly acid to rosolic acid. It remained clear and could 25 be diluted with an equal weight of water without clouding or precipitating the resin. Such a solution may be used in the treatment of cellulose products.

#### Example 4

108 parts cresol, 120 parts formalin, 160 parts water and 3 parts ammonia sp. g. .897 were heated to boiling under a reflux condenser for 30 minutes, after which time the reaction mixture was still a clear liquid. It was then dehydrated until about 140 parts of a viscous resin was obtained still containing about 18% water. This was dissolved in 43 parts of alcohol containing 2 parts lime. The resulting dispersion 35 was clear and could be diluted with at least an equal quantity of water. It could be used with 40 advantage for the treatment of cellulosic materials.

Other resins or resinoids which have, or can 45 be given, a hydrophile character, such as rosin and other natural resins, such as shellac, urea-formaldehyde resinoids, resins of the alkyd type and the like may also be advantageously used in practicing the invention.

#### Example 5

60 parts urea and 160 parts aqueous formaldehyde 40% solution and 1 part hexamethylene tetramine were boiled under a reflux condenser 55 for 15 minutes. The reaction mixture was a clear liquid at the end of the reaction period. 50 parts denatured alcohol were added and 2 parts of citric acid which was sufficient acid to render the liquid resinous mass, just faintly acid 60 to litmus. This liquid resinous mass could be diluted with an equal quantity of water without initiating clouding, if used within three hours after completion of the reaction, and was suitable for use with cellulosic compositions. On 65 standing more than three hours, however, the liquid resinous mass tolerated less and less water.

The hydrophile resinous substances are preferably applied by passing the dried or undried sheet through a bath of the resinous composition 70 or by spraying the resinous composition upon the surface of the dried or undried fibrous sheet. It is particularly advantageous to apply the resinous composition to the undried sheet as in this case one drying operation is eliminated.

For example, the liquid resinous composition may be applied to the paper web as it comes from the wire of a Fourdrinier machine or analogous device. In this case the sheet has typically a 5 water content of about 60% and the liquid resinoid composition immediately penetrates and disappears into the sheet.

When a sheet or a stack of sheets treated as just described is dried and subjected to hot 10 pressing or calendering a most marked and unexpected resistance to moisture absorption is brought about as well as a greatly improved surface appearance.

After treatment of the fibrous sheet with 15 liquid resinoid composition, it is dried. If the composition comprises a resinoid of the heat-hardenable type the drying operation is preferably so carried out that the moisture content is removed without materially advancing the stage 20 of polymerization of the resinoid.

If a laminated product is desired the drying operation is advantageously conducted as follows: The web of treated fibrous material is rolled on a cylinder or similar device until the desired 25 thickness of board is obtained. The board is then cut from the cylinder and dried, preferably by hanging in lofts. After the boards are dried they are subjected to combined heat and pressure between heated platens, whereby well 30 bonded laminated structures of high moisture resistance are produced.

This method provides an effective and economical way of producing laminated structures as it obviates the necessity of coating and superposing a number of separate sheets.

When aqueous resinous compositions containing an organic solvent are used, the proportion of such solvent is preferably limited to such an amount, depending on the particular solvent, 40 that after application of the composition to a fibrous surface and evaporation of the solvent, sufficient water remains to insure proper distribution of the hydrophile resinous content. Enough water should remain after removal of 45 the solvent to prevent undue concentration and agglomeration of the resin. When a water-alcohol mixture is used the alcohol may constitute as much as 90% of the mixture without disturbance of the hydrophile action when it is 50 evaporated. When the residual water is thereafter removed, the resinous substance remains associated with the fiber, apparently in the form of extended films.

The application of hydrophile resinous compositions is not limited to the procedures described above. The compositions can, for example, be sprayed or dripped onto the web just prior to its passage under the "making roll" or onto the sheet as it winds upon the making roll. 60 Another alternative method comprises spraying a partially dried sheet while it is passing through the paper driller, or to apply the resinous composition thereto by means of a contact roller. It is not essential that the paper be in a wet condition, as the resinous composition may be applied to the paper when dry or partially dried; obviously, however, it is usually advantageous to make the application to the sheet while in the wet condition to avoid a second drying.

70 The present invention has been found to be of particular advantage when applied to fibrous sheet material which has had a binding agent,

such as a phenolic resinoid, a resin or other binder, associated therewith in the process of manufacture. An example of such fibrous sheet material which has given particularly desirable results in the present invention are resinoid-containing fibrous sheets produced by the so-called wet process. In a typical form of this process a solid phenolic resinoid in powdered or sludge form is added to the fiber pulp in a beater and thoroughly mixed. The pulp is made into a 10 sheet in the usual manner and dried. If, before drying such sheets, they are treated with a liquid hydrophile resinous composition, for example a phenolic resinoid composition, in the manner described above, laminated structures made by 15 superposing the dried sheets and subjecting the stack to heat and pressure, are found to have greatly reduced water absorption, even when the added resinoid is as low as 0.5% of the sheet. The water absorption is normally reduced to one- 20 tenth or less of its original value by the treatment of the invention, although the added resinoid amounts to only one-third to one twenty-fifth of the resinoid originally present.

Not only is there the marked and unexpected 25 decrease in water absorption of the finished product, due to the application of a hydrophile resinous substance to a resin-containing sheet, but the material produced in accordance with the invention also exhibits a substantial improvement in 30 the surface appearance after molding or hot-pressing into laminated or board stock. An increased uniformity of resin distribution in the body of the material is also obtained. As a result of this improvement hot-pressed laminated 35 structures and other articles produced by the method of the invention can, for example, be sanded without the formation of a striated surface effect such as results from the sanding of laminated material made by the usual method of 40 coating and impregnating sheets with alcoholic or other solutions of resinoids, and removing the solvent.

This application is a continuation-in-part of our application Serial No. 727,582, filed May 25, 45 1934.

We claim:

1. Fibrous composition having incorporated therewith a binder and in addition having uniformly associated with the fibers thereof a hydrophile heat-hardenable phenolic resinoid capable of admixture with up to 70 parts of water per 50 30 parts of the resinoid in neutral condition without clouding or precipitation.

2. Fibrous composition having incorporated therewith a phenolic resinoid binder and in addition having uniformly associated with the fibers thereof a hydrophile heat-hardenable phenolic resinoid capable of admixture with up to 70 parts of water per 60 30 parts of the resinoid in neutral condition without clouding or precipitation.

3. Fibrous composition having incorporated therewith from 15 to 50% of a phenolic resinoid binder and in addition having uniformly associated with the fibers thereof from 0.5 to 10% of 65 a hydrophile heat-hardenable phenolic resinoid capable of admixture with up to 70 parts of water per 30 parts of the resinoid in neutral condition without clouding or precipitation.

CERTIFICATE OF CORRECTION.

Patent No. 2,229,357.

January 21, 1941.

GORDON E. WIGHTMAN, ET AL.

It is hereby certified that error appears in the printed specification of the above numbered patent requiring correction as follows: Page 3, second column, line 51, claim 1, for "heat-hardened" read --heat-hardenable--; and that the said Letters Patent should be read with this correction therein that the same may conform to the record of the case in the Patent Office.

Signed and sealed this 18th day of February, A. D. 1941.

Henry Van Arsdale,

Acting Commissioner of Patents.

(Seal)